

Patented Apr. 13, 1926.

## UNITED STATES PATENT OFFICE.

THOMAS P. SHIELDS, OF NEW YORK, N. Y., ASSIGNOR TO SHIELDS & MOORE, A FIRM  
CONSISTING OF THOMAS P. SHIELDS AND G. A. MOORE, OF NEW YORK, N. Y.

## GOLD ALLOY.

No Drawing.

Application filed July 6, 1925. Serial No. 41,874.

*To all whom it may concern:*

Be it known that I, THOMAS P. SHIELDS, a citizen of the United States, residing at New York city, New York, have invented certain new and useful Improvements in Gold Alloys, of which the following is a specification.

The present invention relates to gold alloys and has for its special object to produce 10 socalled "green gold" as well as socalled "yellow gold" alloys, which alloys can be produced at a low price and in an efficient manner.

A special object of the invention is to produce 15 a gold alloy of the character specified, which will melt at such temperatures as are readily secured by goldsmiths with the same heating appliances used in melting pure gold and its common alloys such as those ordinarily used in making jewelry, etc. In my copending application, I describe alloys 20 of the class above identified, and containing chromium as a constituent, but such alloys, especially when containing over about 2% chromium are more difficult to melt.

The invention will be described in connection with several specific examples, but it is to be understood that the invention is not restricted to these specific examples.

30 In the preferred form of the invention, I first preferably prepare an alloy of chromium, copper and zinc (with or without silver) in desired proportions, as given below (termed alloying alloy), to which I then add, while said alloy is molten a sufficient amount of gold (e. g. fine gold or gold containing some alloying metals as commonly found in the market) to bring the total actual gold content up to say 40 to 60% of the whole.

40 As examples of the "alloying alloy" I give the following:

*Example 1.*

45 .1 parts to 1 part chromium, 24 parts to 50 parts copper, 10 parts to 30 parts zinc, 5 parts to 15 parts silver.

*Example 2.*

50 0.8 parts to 2 parts chromium, 24 parts to 50 parts copper, 10 parts to 18 parts zinc.

These alloys, in a molten state, are then mixed with melted gold, as above stated, the latter amounting to 40 to 60% of the entire

alloy to form finished alloys, say of the following composition. Preferably the chromium is not substantially over 1% and in all cases is less than 2% of the finished alloy.

*Example 3.*

40% to 60% gold, together with 60 to 40% of an alloy consisting of 24 to 50 parts of copper, 10 to 35 parts of zinc, 00 to 15 parts of silver, 0.1 to 1 part of chromium.

*Example 4.*

40% to 60% gold, together with 60 to 40% of an alloy consisting of .8 to 1 part of chromium, 20 to 50 parts of copper, 10 to 35 parts of zinc.

These alloys have most of the properties of the other alloys of Serial No. 31,671. The difference is that a part of the chromium is replaced by zinc.

I then can cast this alloy into desired shapes or can roll out the same into sheets or draw it into rods, wire or other forms.

In compounding the final alloy from "alloying alloy" and gold which already contains substantial amounts of other metals, it is of course possible to take the latter into consideration when making up the "alloying alloy", for that particular batch.

It will be understood that the presence of metals other than those above mentioned, in small amounts in the final alloy, is not precluded. Such other metals, if present in substantial amounts may of course influence the properties of the alloy, to a greater or less extent.

*Example 5.*

I employ about 58.3% of fine gold, 0.5% of chromium, 2% of fine silver, 14% of zinc and 25.2% of copper. This produces an alloy which is relatively low in gold, but possesses the property of not readily tarnishing, and this alloy will be found to have the desired "green gold" color and will have good working properties. It is fusible at about the same temperature as gold. This alloy is very cheap to produce, and can be readily worked with ordinary goldsmiths' tools, and also can be readily enameled.

In this example, as in several of the other examples, the amount of silver can be greatly reduced, and if desired can be omitted altogether, and if it is desired to decrease the

amount of silver it is preferable to increase the amount of chromium somewhat.

*Example 6.*

5 40% of fine gold, 1% of chromium, 30% of copper, 29% of zinc and no silver are employed. In this alloy it is noted that the amount of gold is relatively low so that the alloy is cheaply produced, and is very suitable for making up jewelry.

In making up the alloy, I preferably mix together the chromium, copper and zinc (and silver if it is to be used) in about the proportion in which they are to exist in the final alloy. These metals can be mixed together, melted and granulated, to form an "alloying" alloy, and the desired amount of this is added to the desired amount of fine gold, (or gold which may contain common alloying 15 metals, e. g. copper) so as to give the percentage of gold desired, and again melted and stirred, to give the desired final product.

The final alloys, as will be noted, do not 25 contain any of the metals of the platinum group, which have heretofore been used in alloys of this general class, for the prevention

of tarnishing. The metals of this group however are extremely expensive, and I find that the alloys produced in accordance with the present invention are substantially free from tendency to tarnish, even in the form of jewelry about 10 to 14 carat.

I claim:—

1. An intermediate alloy consisting essentially of:—chromium 0.1 to 2 parts, copper 24 to 50 parts, and zinc 10 to 18 parts.

2. An intermediate alloy consisting essentially of:—chromium 0.1 to 2 parts, copper 24 to 50 parts, zinc 10 to 18 parts, and silver 40 not over 15 parts.

3. A gold alloy consisting essentially of 40 to 60% gold, together with 60 to 40% of an alloy of 0.1 to 2 parts of chromium, 20 to 50 parts of copper, and 10 to 35 parts of 45 zinc.

4. A gold alloy consisting essentially of 40 to 60% gold, together with 60 to 40% of an alloy of 0.1 to 2 parts of chromium, 20 to 50 parts of copper, 10 to 35 parts of zinc, and 50 silver in some amount not substantially above 15 parts.

In testimony whereof I affix my signature.

THOMAS P. SHIELDS.